

2,954,344

## HEAVY DUTY LUBRICATING OIL

James R. Miller, Baytown, Tex., assignor, by mesne assignments, to Esso Research and Engineering Company, Elizabeth, N.J., a corporation of Delaware

No Drawing. Filed Dec. 11, 1957, Ser. No. 701,980

3 Claims. (Cl. 252—33.4)

The present invention is directed to an improved lubricating oil. More particularly, the present invention is directed to a lubricating oil composition suitable for use under heavy duty conditions. In its more specific aspects, the invention is directed to a useful lubricating oil having improved stability characteristics.

The present invention may be briefly described as a lubricating oil composition of improved stability which comprises synergistic amounts of an orthoalkylated phenol and an alkaline earth metal sulfonate in admixture with a lubricating oil fraction.

The lubricating oil fraction employed in the practice of the present invention may suitably be a paraffinic or naphthenic type lubricating oil, such as produced from Gulf Coastal, Panhandle, and Pennsylvania and California type crude oil. The lubricating oil fraction may suitably have a range in viscosity from about 35 to about 160 Saybolt Seconds Universal at 210° F. While the lubricating oil fraction is preferably a petroleum lubricating oil fraction, other lubricating oils may be employed in the composition of the present invention. Thus, lubricating oils produced synthetically by polymerizing olefins to oils of the proper molecular weight and having lubricating oil characteristics in the viscosity range indicated may be used.

The amount of the composition made up of the lubricating oil fractions will suitably be in the range from about 93 percent to about 98 percent by weight of the composition.

The composition contains synergistic amounts of an orthoalkylated phenol and an alkaline earth metal sulfonate. The orthoalkylated phenol is suitably an orthoalkylated phenol such as 2,6 di-tertiary butyl phenol, 2,6 di-tertiary- $\alpha$ -dimethylamine para-cresol, 4,4'-methylenebis (2,6-di-tertiary butyl phenol), ortho-tertiary butyl phenol, and 2,4,6 tri-tertiary butyl phenol.

The amount of the orthoalkylated phenol employed suitably ranges between about 0.5 percent and about 2 percent by weight of the composition.

The alkaline earth metal sulfonate may be any of three alkaline earth metal sulfonates, such as calcium, barium, or strontium, but preferably is calcium or barium sulfonate. These alkaline earth sulfonates may be suitably formed by alkylating benzene with tetrapropylene to form a long chain alkylated aromatic hydrocarbon, followed by sulfonation of the alkylated hydrocarbon, and then neutralizing the sulfonated alkylated aromatic hydrocarbon with barium or calcium hydroxide or oxide. Other means for preparing the sulfonate may be employed, for example, by photosulfochlorination of saturated hydrocarbons with corresponding treatment of the sulfonyl chloride with barium or calcium oxide or hydroxide.

The synergistic amount of the alkaline earth sulfonate is between about 1 percent and about 5 percent by weight of the composition.

The alkaline earth sulfonate may contain a co-neutralized alkyl phenate in admixture with the alkaline

earth metal sulfonate. When a co-neutralized alkyl phenate is employed, it should be employed with the alkaline earth metal sulfonate in a ratio of two parts of the alkaline earth metal sulfonate to about 1 part of the co-neutralized alkyl phenate.

As examples of the alkyl phenates may be mentioned nonyl barium phenate, sulfurized nonyl barium phenate, sulfurized calcium-barium nonyl phenate, and sulfurized calcium nonyl phenate.

10 In order to illustrate the present invention further a number of compositions were made up in accordance with the present invention in which synergistic amounts of the orthoalkylated phenol and the alkaline earth metal sulfonate were employed. These compositions were compared with other compositions employing the orthoalkylated phenol and the alkaline earth metal sulfonate alone. Further comparisons were made with compositions of the prior art.

The several blends were subjected to a modified Indiana 20 Life test for 32 hours and the percent increase in viscosity (Saybolt Seconds Universal) at 100° F. was established by determining the viscosity every 8 hours and plotting percent viscosity increase versus time. Identity of the several blends and the results of the Indiana Life 25 test are presented in the following table:

Table I

| Blend No. | Additive                                                                                                                                                            | Percent Viscosity Increase (After 32 Hours in Modified Indiana Life Test) |
|-----------|---------------------------------------------------------------------------------------------------------------------------------------------------------------------|---------------------------------------------------------------------------|
| 30        |                                                                                                                                                                     |                                                                           |
| 1.....    | Base+0.5 Wt. Percent 4,4' Methylenebis (2,6-di-tert-butyl phenol).                                                                                                  | 35                                                                        |
| 2.....    | Base+0.75 Wt. Percent 4,4' Methylenebis (2,6-di-tert-butyl phenol).                                                                                                 | 32                                                                        |
| 3.....    | Base+1.0 Wt. Percent 4,4' Methylenebis (2,6-di-tert-butyl phenol).                                                                                                  | 30                                                                        |
| 4.....    | Base+1.5 Wt. Percent 4,4' Methylenebis (2,6-di-tert-butyl phenol).                                                                                                  | 26                                                                        |
| 5.....    | Base+0.5 Wt. Percent 2,6-di-tert-butyl- $\alpha$ -dimethylamine-p-cresol.                                                                                           | 35                                                                        |
| 40        | Base+1.0 Wt. Percent 2,6-di-tert-butyl- $\alpha$ -dimethylamine-p-cresol.                                                                                           | 32                                                                        |
| 6.....    | Base+1.5 Wt. Percent 2,6-di-tert-butyl- $\alpha$ -dimethylamine-p-cresol.                                                                                           | 30                                                                        |
| 7.....    | Base+2.5% sulfurized nonyl barium phenate.                                                                                                                          | 29                                                                        |
| 8.....    | Base+5.0% 1 part calcium sulfonate, 2 parts co-neutralized sulfurized nonyl calcium-barium phenate.                                                                 | 23                                                                        |
| 45        |                                                                                                                                                                     |                                                                           |
| 9.....    | Base+2.5% 2 parts barium sulfonate, 1 part co-neutralized sulfurized nonyl calcium-barium phenate.                                                                  | 34                                                                        |
| 10.....   | Base+4.0% Ca Sulfonate.                                                                                                                                             | 35                                                                        |
| 11.....   | Base+2.5% Ba Sulfonate.                                                                                                                                             | 50                                                                        |
| 12.....   | Base+2.5% sulfurized nonyl barium phenate, 1.0% 4,4' Methylenebis (2,6-di-tert-butyl phenol) (Wt.).                                                                 | 24                                                                        |
| 50        |                                                                                                                                                                     |                                                                           |
| 13.....   | Base+5.0% 1 part calcium sulfonate, 2 parts co-neutralized sulfurized nonyl calcium-barium phenate; 1.0% 4,4' Methylenebis (2,6-di-tert-butyl phenol) (Wt.).        | 22                                                                        |
| 14.....   | Base+5.0% 1 part calcium sulfonate, 2 parts co-neutralized sulfurized nonyl calcium-barium phenate; 1.0% 4,4' Methylenebis (2,6-di-tert-butyl phenol) (Wt.).        | 24                                                                        |
| 15.....   | Base+5.0% 1 part calcium sulfonate, 2 parts co-neutralized sulfurized nonyl calcium-barium phenate; 1.0% 2,6-di-tert-butyl- $\alpha$ -dimethylamine-p-cresol (Wt.). | 24                                                                        |
| 55        |                                                                                                                                                                     |                                                                           |
| 16.....   | Base+2.5% 2 parts barium sulfonate, 1 part co-neutralized sulfurized nonyl calcium-barium phenate; 1.0% 4,4' Methylenebis (2,6-di-tert-butyl phenol) (Wt.).         | 14                                                                        |
| 17.....   | Base+2.5% 2 parts barium sulfonate, 1 part co-neutralized sulfurized nonyl calcium-barium phenate; 1.0% 2,6-di-tert-butyl- $\alpha$ -dimethylamine-p-cresol (Wt.).  | 18                                                                        |
| 60        |                                                                                                                                                                     |                                                                           |
| 18.....   | Base+4.0% Ca Sulfonate, 1.0% 4,4' Methylenebis (2,6-di-tert-butyl phenol) (Wt.).                                                                                    | 15                                                                        |
| 19.....   | Base+2.5% Ba Sulfonate, 1.0% 4,4' Methylenebis (2,6-di-tert-butyl phenol) (Wt.).                                                                                    | 15                                                                        |
| 20.....   | Base+2.5% 2 parts barium sulfonate, 1 part co-neutralized sulfurized nonyl calcium-barium phenate; 0.75% 4,4' Methylenebis (2,6-di-tert-butyl phenol) (Wt.).        | 14                                                                        |
| 65        |                                                                                                                                                                     |                                                                           |
| 21.....   | Base+2.5% 2 parts barium sulfonate, 1 part co-neutralized sulfurized nonyl calcium-barium phenate; 0.5% 4,4' Methylenebis (2,6-di-tert-butyl phenol) (Wt.).         | 14                                                                        |
| 70        |                                                                                                                                                                     |                                                                           |

From the data presented in the preceding table, it will be clear that the blends containing both the alkaline earth

metal sulfonate and the orthoalkylated phenol showed less increase in viscosity than the blends containing only the orthoalkylated phenol or the calcium sulfonate. Further, it is to be noted that blend No. 13, which contained both sulfurized nonyl barium phenate and ortho-alkylated phenol, showed an increase in viscosity of 24 against an increase in viscosity of 29 for blend No. 8, which contained only the sulfurized nonyl barium phenate. It is to be noted that neither blend 8 nor blend 13 contained any of the alkaline earth sulfonate. Furthermore, comparing blend 13 with blend 14, where the mixture of calcium sulfonate and co-neutralized sulfurized nonyl calcium-barium phenate, having a ratio of 1:2, was employed, a synergistic effect was not noted. This is also evidenced by blend No. 15. On the other hand, blend No. 10, where two parts of barium sulfonate and one part of co-neutralized sulfurized nonyl calcium-barium phenate was used, a viscosity increase of 34 was realized and when this material was used with the ortho-alkylated phenol, as shown in blends 16 and 18, a synergistic effect was noted. This effect is also shown in blends 20 and 21.

From the data presented in the table, it may be concluded that the alkaline earth metal sulfonate should be employed with the co-neutralized sulfurized alkyl phenate in a ratio of two parts of the alkaline earth metal sulfonate to one part of the phenate to obtain the synergistic effect when employed with the orthoalkylated phenol.

The Indiana Life test employed to show the beneficial effects of the present invention is described in The Journal of Industrial and Engineering Chemistry, Analytical Edition, vol. 6, page 419, by Rogers and Shoemaker. The Modified Indiana Life test consists in suspending a rod having strips of copper, iron and zinc wrapped thereon in the oil during the oxidation period and the withdrawal of samples of sufficient amount at specified intervals for determination of viscosity from which the viscosity increase is calculated.

The present invention is quite useful in that heavy duty lubricating oil possessing outstanding cleanliness, anti-

wear and stability characteristics is provided for use in lubricating internal combustion and other types of engines subjected to heavy duty. The lubricating oil composition in accordance with the present invention is quite useful when employed in lubricating engines such as those of the Chevrolet type possessing outstanding stability and cleanliness.

The nature and objects of the present invention having been completely described and illustrated, what I wish to claim as new and useful and to secure by Letters Patent is:

1. A lubricating oil composition of improved stability which consists of synergistic amounts in the range between about 0.5% and about 2.0% by weight of an orthoalkylated phenol consisting of 2,6 tertiary butyl  $\alpha$  dimethyl amine para-cresol, between about 1% and about 5% by weight of an alkaline earth metal sulfonate inhibitor containing a co-neutralized sulfurized nonyl phenate, said alkaline earth metal sulfonate and co-neutralized sulfurized nonyl phenate being in a ratio of about 2:1, and between about 93% and about 98.5% by weight of a lubricating oil.

2. A composition in accordance with claim 1 in which the alkaline earth metal is calcium.

25 3. A composition in accordance with claim 1 in which the alkaline earth metal is barium.

#### References Cited in the file of this patent

#### UNITED STATES PATENTS

|    |           |                        |                |
|----|-----------|------------------------|----------------|
| 30 | 2,270,577 | Bergstrom et al. ----- | Jan. 20, 1942  |
|    | 2,410,652 | Griffin et al. -----   | Nov. 5, 1946   |
|    | 2,629,693 | Barton et al. -----    | Feb. 24, 1953  |
|    | 2,652,367 | Adelson -----          | Sept. 15, 1953 |
| 35 | 2,693,448 | Landis et al. -----    | Nov. 2, 1954   |
|    | 2,695,273 | Hook et al. -----      | Nov. 23, 1954  |
|    | 2,750,340 | Gerhardt et al. -----  | June 12, 1956  |

#### FOREIGN PATENTS

|                     |               |
|---------------------|---------------|
| Canada -----        | Nov. 24, 1953 |
| Great Britain ----- | Aug. 24, 1948 |